

J. C. RUSSELL.  
PROCESS OF UNITING METALS.  
APPLICATION FILED DEC. 30, 1912.

1,090,088.

Patented Mar. 10, 1914.

2 SHEETS-SHEET 1.

Fig. 1.



Fig. 2.



Fig. 3.



Fig. 4.



Fig. 5.



Fig. 6.



WITNESSES

W. C. Cooke  
B. J. Brooke

INVENTOR

James C. Russell  
By J. C. Cooke,  
attorney.

J. C. RUSSELL.  
PROCESS OF UNITING METALS.  
APPLICATION FILED DEC. 30, 1912.

1,090,088.

Patented Mar. 10, 1914.

2 SHEETS—SHEET 2.



*Fig. 8.*



*Fig. 10.*



*Fig. 9.*



WITNESSES

W. G. Cooke  
B. J. Brooke

INVENTOR

James C. Russell  
By J. M. Cooke  
Attorney.

# UNITED STATES PATENT OFFICE.

JAMES C. RUSSELL, OF PITTSBURGH, PENNSYLVANIA.

## PROCESS OF UNITING METALS.

1,090,088.

Specification of Letters Patent. Patented Mar. 10, 1914.

Application filed December 30, 1912. Serial No. 739,190.

To all whom it may concern:

Be it known that I, JAMES C. RUSSELL, a resident of Pittsburgh, in the county of Allegheny and State of Pennsylvania, have 5 invented a new and useful Improvement in Processes of Uniting Metals; and I do hereby declare the following to be a full, clear, and exact description thereof.

My invention relates to the treating of 10 metal articles and has special reference to the treatment of amalgamated or combined metals in an ingot form.

The object of my invention is to provide 15 a cheap, simple and efficient grade of sheets, plates, bars, wire, etc., having an interior of steel and an exterior of copper or copper alloy wherein such interior and exterior will be completely amalgamated at their joining point in order to form a solid homogeneous mass of metal, and also a finished 20 product of combined metal which will be entirely free from any flaws or blow-holes on account of the segregation being prevented in the rotating or spinning of the 25 metal while in ingot form.

My invention consists, generally stated, in the novel method as hereinafter more specifically set forth and described and particularly pointed out in the claims.

To enable others skilled in the art to which my invention appertains to carry out and use my improved process I will describe the same more fully referring to the accompanying drawings, in which:—

Figure 1 is a longitudinal sectional view of the apparatus used in carrying out my improved process of amalgamating metals. Fig. 2 is a cross sectional view of the same showing the parts in the pit in full lines. Fig. 3 is a vertical sectional view of an ingot mold showing the molten metal therein. Figs. 4, 5 and 6 are vertical sectional views of the finished material. Fig. 7 shows a cross sectional view of an apparatus for treating hollow ingots. Fig. 8 is a cross sectional view of the hollow ingot in the ingot mold. Fig. 9 is a longitudinal sectional view of the ingot after treatment in the rolls. Fig. 10 is a modified form of ingot 50 mold.

Like symbols of reference herein indicate like parts in each of the figures of the drawings.

As illustrated in the drawings my improved process is carried on in the ingot mold *a* and in the apparatus *b*. The ingot

mold *a* is formed of the ordinary material and has a slight taper so that it is smaller at the bottom than at the top, and it is preferably made in two parts in order that it may be clamped together to receive a tube as hereinafter explained.

The process herein described is similar to the process described in my U. S. Letters-Patent. No. 1,019,191 granted March 5th, 1912, for an improvement in treating metal articles.

The apparatus *b* used in my improved process of combining metals has side frames or housings 1 in which are journaled the lower rolls 2 and 3 and the upper rolls 4 and 5 and such lower rolls are not adapted to be moved in a vertical direction as the adjustment of the distance between the upper and lower rolls is obtained by means of the vertical movement of the upper rolls 4 and 5. The upper rolls 4 and 5 are journaled in sliding bearings 6 located in the housings 1, as shown in Fig. 1. Below the rolls 2 and 3 and housings 1 is a pit 7 into which rods 8 extend and such rods are connected at their upper ends to the sliding bearings 6 and at their lower ends to a bar 9. This bar 9 is connected at its center or any convenient place with the cross bar 10 which is hung or pivoted at its center from the supporting shoulder 11 which extends downward from the base plate 12. The outer end of the cross bar 10 is fastened to a heavy counter weight 13 by any suitable means and such weight is adapted to be moved vertically by the cross bar 10 on its pivotal connection 14 while a rod 15 extending between the bottom of the pit 7 and the base plate 12 and through the said counter weight guides the same in its vertical movement. The upper rolls 4 and 5 are adapted to be controlled by means of screws 16 which extend down from the top of the frames 1 and bear upon the upper part of the sliding bearings 6 while each of said screws is provided at its upper end with a bevel gear 17 which meshes with gears 18 on the horizontal shaft 19 and such shaft is operated by means of a hand-wheel or bar 20 at one end of the same.

The machine is provided with the front and rear tables 21 and 22 for the purpose of admitting and discharging the ingots *c* from the rolls as hereinafter described. The rolls 2, 3, 4 and 5 are each provided with slots or grooves 23, which extend around the cir-

5 circumference of the same and form flanges 24 while an idle roll or disk 25 is adapted to rest in said grooves, as later explained. The idle roll or disk 25 on one side of the rolls 2, 3, 4 and 5 is provided with an opening 26 in the same through which a plunger 27 is adapted to extend and such plunger is connected at its outer end to an accumulator or other apparatus (not shown), as later described. The inner end of the plunger 27 is provided with a small roller 27<sup>a</sup> which is adapted to bear against and rotate with the ingot as it is rotated between the rolls 2, 3, 4 and 5.

15 My improved process of amalgamating metals is as follows: I first take a piece of sheet or plate metal such as copper, or any other metal or an alloy, and fit the same into the ingot mold *a* after uniting the side edges 20 of the same by means of an acetylene torch or other means and such sheet will then form a tube 28 which will exactly fit the interior of the mold *a*. The molten metal is now poured into the mold in order to fill up 25 the interior of the tube 28 precisely the same as though the interior of such tube were the interior of the mold *a*. This operation will cause the molten metal to fuse the inner part of the tube 28 and thus become amalgamated with the same while the outside 30 of such tube will become plastic but will not fuse or assume a liquid state. The ingot is now taken from the mold as the ends of the same soon become frozen and is carried to 35 the rolling apparatus *b* where it is inserted in the rolls 2, 3, 4 and 5 and such rolls are rotated at a rapid rate of speed by any suitable means. The ingot *c* thus formed is 40 of conical shape and is in a liquid condition in its center while the outside is covered by the tube 28 which is now in a plastic condition and the ends are solidified just sufficient to prevent the liquid metal in the 45 interior of the ingot from escaping therefrom. The larger end of the ingot is held against the disk or roll 25 by means of the small plunger 27 which has the roller 27<sup>a</sup> on its end and which bears against the smaller end of such ingot with the pressure 50 exerted by the accumulator which is adjusted to give just sufficient pressure to hold the ingot in place without bearing hard enough to prevent the necessary elongation. As the rolls thus engage the larger end of 55 the ingot *c* such ingot will be decreased in diameter and the gases collected in the same will be forced out from the sides thereof so that the whole when finished will be a solid homogeneous mass. This elimination 60 is accomplished by reason of the inner part of the ingot being in a liquid form so that when the same is rotated the liquid will be gathered up into the plastic or pasty material much the same as in the puddling process and as the rolls bear upon the outer sur-

face of the same the gases will be forced out through the same so that all the blow-holes, pipe and segregation will be eliminated and the finished ingot will be a solid homogeneous mass covered with an outer 70 coating of copper or other metal which will be amalgamated with the inner metal and no joining or break line will be apparent.

Fig. 1 shows a hood 29 in dotted lines and such hood is for the purpose of retaining 75 heat in case the ingot becomes chilled as at such times heat is applied to the outer surface of the same by means of gas jets or acetylene burners. After the ingot *c* is taken from the apparatus *b* by raising the upper 80 rolls 4 and 5 it is pressed either into billets 30, as shown in Fig. 5, or rolled into sheets 31, as shown in Fig. 6. These sheets 31 will be coated with a thin covering of copper or other metal and the thickness of such coating will depend upon the thickness to which the inner metal is rolled out. If desired the reduced ingot after being taken from the spinning rolls may be subjected to a squeezing operation in any apparatus, so 85 that pressure will be exerted upon the outer surface of the same as it cools to atmospheric temperature for the purpose of assisting the molecules comprising the same in becoming firmly bonded together. By using copper 90 and various amounts of nickel as an alloy in making the tube 28 the outside of the finished material will be from dark bronze to a white metal. Any metal or alloy which is non-corrosive or rustless may be used on 100 the outside of the ingot for making the combination metal, and these may all be applied in the manner described.

It will be evident that the production of metal by my improved process can be used 105 in the same places where copper coated metal is used at the present day and will also take the place of solid copper in many instances where it is necessary to have a rustless material. It will be very useful in sheet 110 roofing as copper is very expensive and other metals will not stand the exposure to the weather. It can be made almost as cheap as galvanized steel so that it will decrease the cost of copper plated material and render its 115 use practical in places where its high cost has heretofore made its use prohibitive.

In referring to Figs. 7, 8, 9 and 10 of the drawing these figures illustrate the method employed in making hollow metal ingots 120 wherein the inner surface material is different than the body of the ingot and is united therewith to form a solid homogeneous mass. In forming hollow ingots the ingot mold *M*, in which the same are formed 125 has a projection 28' in the bottom of the same upon which a pipe or tube 29' is placed, the upper end of such tube extending to the height to which the molten metal is to be poured. The molten metal is now poured 130

into the ingot mold and around the tube 29' so that such tube, which is of copper, copper alloy or other metal, will become fused or amalgamated with the metal of the ingot body. The ingot may be made as large as desired as may also the hollow center of the same. As soon as the ingot becomes frozen on the outside of the same it is carried to the apparatus K used for treating hollow ingots and such apparatus is exactly the same as the apparatus used for the solid ingots except that a rod 30 extends through one of the idle disks or side rolls 25 and through the hollow interior of the ingot and such rod will rotate with the ingot and keep the hollow center of the same from being crushed in during the rolling operation. In this connection it will be seen that ingots thus formed may have an inside and an outside of copper or copper alloy and the body of the same formed of a homogeneous mass of steel.

Various modifications and changes in the process of treating my improved metal article may be resorted to without departing from the spirit of the invention or sacrificing any of its advantages.

What I claim as my invention and desire to secure by Letters-Patent, is:—

30 1. The herein described process of forming combined metal ingots to prevent blow-holes, segregation and the injurious action of the pipe formed therein, which comprises the steps of introducing molten metal 35 against another metal in an ingot mold in order to form an ingot circular in cross section, said molten metal heating said other metal to a semi-plastic condition, and then applying pressure to the side of such ingot 40 to reduce the same and force the gases therefrom while rotating the ingot about its longitudinal axis.

2. The herein described process of forming combined metal ingots to prevent blow-holes, segregation and the injurious action 45 of the pipe formed therein, which comprises the steps of introducing molten metal against another metal in an ingot mold in order to form an ingot into conical shape 50 and circular in cross section, said molten metal heating said other metal to a semi-plastic condition, and then applying pressure to the side of such ingot to reduce the same and force the gases therefrom while 55 the ingot is being subjected to a spinning movement about its longitudinal axis.

3. The herein described process of forming combined metal ingots to prevent blow-holes, segregation and the injurious action 60 of the pipe formed therein, which comprises the steps of introducing molten metal against a tube of another metal in an ingot mold in order to form an ingot circular in cross-section, said molten metal heating said 65 other metal to a semi-plastic condition, and

then applying pressure to the side of such ingot to reduce the same and force the gases therefrom while rotating the ingot about its longitudinal axis.

4. The herein described process of forming hollow ingots of combined metals to prevent blow-holes, segregation and the injurious action of the pipe formed therein, which comprises the steps of introducing molten metal around a tube of another metal in an ingot mold in order to form an ingot circular in cross section, said molten metal heating said other metal to a semi-plastic condition, and then applying pressure to the sides of such ingot to reduce the same and force the gases therefrom while rotating the ingot about its longitudinal axis. 70 75 80

5. The herein described process of forming hollow ingots of combined metals to prevent blow-holes, segregation and the injurious action of the pipe formed therein, which comprises the steps of introducing molten metal around a tube of another metal in order to form an ingot circular in cross section, and then applying pressure to the sides of such ingot to reduce the same and force the gases therefrom while rotating the ingot about its longitudinal axis while holding the hollow center to prevent the same from being crushed under such pressure. 85 90 95

6. The herein described process of forming combined metal ingots to prevent blow-holes, segregation and the injurious action of the pipe formed therein, which comprises the steps of introducing molten metal 100 against another metal in an ingot mold in order to form an ingot circular in cross section, then applying pressure to the side of such ingot to reduce the same and force the gases therefrom while rotating the ingot about its longitudinal axis, and then squeezing the reduced ingot until cold to allow the molecules to become firmly bonded. 105

7. The herein described process of forming combined metal ingots to prevent blow-holes, segregation and the injurious action of the pipe formed therein, which comprises the steps of introducing molten metal against another metal in an ingot mold in order to form an ingot into conical shape 110 and circular in cross section, then applying pressure to the side of such ingot to reduce the same and force the gases therefrom while the ingot is being subjected to a spinning movement about its longitudinal axis, 115 and then squeezing the reduced ingot until cold to allow the molecules to become firmly bonded. 120

8. The herein described process of forming combined metal ingots to prevent blow-holes, segregation and the injurious action of the pipe formed therein, which comprises the steps of introducing molten metal against a tube of another metal in an ingot mold in order to form an ingot circular in 125 130

cross section, then applying pressure to the side of such ingot to reduce the same and force the gases therefrom while rotating the ingot about its longitudinal axis, and then squeezing the reduced ingot until cold to allow the molecules to become firmly bonded.

9. The herein described process of forming combined metal ingots to prevent blow-holes, segregation and the injurious action 10 of the pipe formed therein, which comprises the steps of introducing molten metal against a tube of another metal in an ingot mold in order to form an ingot into conical shape and circular in cross section, then applying pressure to the side of such ingot to reduce the same and force the gases therefrom while the ingot is being subjected to a spinning movement about its longitudinal axis, and then squeezing the reduced ingot 15 until cold to allow the molecules to become firmly bonded.

10. The herein described process of forming hollow ingots of combined metals to prevent blow-holes, segregation and the injurious action of the pipe formed therein, which comprises the steps of introducing molten metal around a tube of another metal in an ingot mold in order to form an ingot circular in cross section, then applying 20 pressure to the sides of such ingot to reduce the same and force the gases therefrom while rotating the ingot about its longitudinal axis, and then squeezing the reduced ingot until cold to allow the molecules to become 25 firmly bonded.

11. The herein described process of forming hollow ingots of combined metal to prevent blow-holes, segregation and the injurious action of the pipe formed therein, which 30 comprises the steps of introducing molten metal around a tube of another metal in an ingot mold in order to form an ingot into conical shape and circular in cross-section, then applying pressure to the sides of such 35 ingot to reduce the same and force the gases

therefrom while the ingot is being subjected to a spinning movement about its longitudinal axis, and then squeezing the reduced ingot until cold to allow the molecules to become firmly bonded.

12. The herein described process of forming hollow ingots of combined metals to prevent blow-holes, segregation and the injurious action of the pipe formed therein, which comprises the steps of introducing 50 molten metal around a tube of another metal mold in order to form an ingot circular in cross section, then applying pressure to the sides of such ingot to reduce the same and force the gases therefrom while rotating the ingot about its longitudinal axis while holding the hollow center to prevent the same from being crushed under such pressure, and then squeezing the reduced ingot 55 until cold to allow the molecules to become 60 firmly bonded.

13. The herein described process of forming hollow ingots of combined metal to prevent blow-holes, segregation and the injurious action of the pipe formed therein, which 70 comprises the steps of introducing molten metal around a tube of another metal in an ingot mold in order to form an ingot into conical shape and circular in cross section, then applying pressure to the sides of such 75 ingot to reduce the same and force the gases therefrom while the ingot is being subjected to a spinning movement about its longitudinal axis while holding the hollow center to prevent the same from being crushed under such pressure, and then squeezing the reduced ingot until cold to allow the molecules to become 80 firmly bonded.

In testimony whereof, I, the said JAMES C. RUSSELL, have hereunto set my hand.

JAMES C. RUSSELL.

Witnesses:

T. B. HUMPHRIES,  
J. N. COOKE.